

May 8, 1973

R. A. PARIS ET AL

3,732,091

METHOD FOR PREPARING MUTUAL DISPERSIONS OF CARBIDES AND METALS  
OR ALLOYS AND NOVEL PRODUCTS THEREOF

Filed July 1, 1970

*Fig. 1.*



*Fig. 2.*



INVENTORS

RENE ANTOINE PARIS  
DOMINIQUE THIBAUDON  
MARC PIERRE ROUBIN  
JACQUES MAURICE PARIS

BY

*William A. Stokes*

ATTORNEY

**1**

3,732,091

**METHOD FOR PREPARING MUTUAL DISPERSIONS OF CARBIDES AND METALS OR ALLOYS AND NOVEL PRODUCTS THEREOF**

René A. Paris and Dominique Thibaudon, Lyon, Marc P. Roubin, Villeurbanne, and Jacques M. Paris, Lyon, France, assignors to Agence Nationale de Valorisation de la Recherche (ANVAR), Puteaux, France

Filed July 1, 1970, Ser. No. 51,470

Claims priority, application France, July 4, 1970,  
6922753

Int. Cl. B22f 9/00

U.S. Cl. 75—5 AC

9 Claims

**ABSTRACT OF THE DISCLOSURE**

A mixed oxide, a co-precipitate of hydroxides or a mixed complex of a first metal providing the carbide of the dispersion and of a second metal providing the metal of the dispersion are subjected to a heat treatment in an enclosure. The compound thus obtained is subjected, in a reducing and carburizing atmosphere containing hydrogen and methane, to thermal treatment below 1100° C. to reduce all the oxides and carburize the first metal. Heating is effected at a speed of 100 to 400° C./hour. The dispersions comprise particles of single or mixed carbides uniformly distributed in the midst of elementary grains of metal. The dispersions are used in powder metallurgy.

The invention relates to a method for the preparation of mutual dispersions of carbides and of metals or alloys, and to the products thereof.

According as the metal or the carbide are preponderant in the dispersion considered, the description will relate to a dispersion of carbide in the metal or a dispersion of metal in carbide.

The dispersions of the first of these two categories have, with respect to the base metal or alloy, strengthened mechanical properties, particularly as regards hardness and resistance to flow, especially at high temperature.

In dispersions of the second of the said categories, the metal serves as binder between the grains of a powder of carbide intended for sintering. Of course, there is also produced an improvement in the mechanical properties of the sintered parts.

The invention relates also to dispersions of single or mixed carbides in metals or alloys having characteristics which make them novel industrial products.

It is a particular object of the invention to make available to industry a method of preparation which is easy to put into practice and which ensures constant quality of the products obtained.

The method according to the invention is characterized in that,

In a first step, there is prepared a mixed oxide, a co-precipitate of hydroxides or a mixed complex of a first metal (or several if it is desired to obtain a mixed carbide) intended to provide the carbide of the dispersion and selected from among Ti, V, Nb, Ta and Cr and of a second metal (or several if it is desired to obtain an alloy) intended to provide the metal of the dispersion and selected from among Fe, Co, Ni, Cu, Zn, Cd, Ag, Sn, Pb, Bi, Ge and Tl, and

In a second step, the compound thus obtained is subjected, in the midst of an atmosphere both reducing and carburizing and comprising hydrogen and a hydrocarbon such as methane, to a heat treatment of which the tem-

**2**

perature (less than 1100° C.) and the duration are selected so that the reduction of all the oxides and the carburization of the first metal are ensured, the heating being effected preferably at a speed of the order of 100 to 400° C./hour.

The dispersions according to the invention of carbides in metals are characterised in that they comprise particles of a single or mixed carbide distributed uniformly in the midst of elementary grains of the metal or alloy selected.

10 In these products, the dimensions of the particles of the disperse phase (which are not concentrated at the junctions of grains of the metallic phase but distributed uniformly inside the latter) are of the order of 5 to 500  $\mu$ .

15 In the case of dispersions of a metal or alloy in a carbide, the metal occurs localised at the junctions of the grains of carbide. Here again, the dimensions of the particles before sintering are of the order of 5 to 500  $\mu$ .

When it is desired that the metallic phase be constituted by an alloy, there is employed a mixed oxide of metals of the second group.

In the case where the carbide of the second metal is stable under the conditions of simultaneous carburation and reduction, this step is followed by a supplementary treatment of reduction in pure hydrogen at the same temperature for a time sufficient to completely reduce the carbide of the said second metal.

The method according to the invention may be applied in a fixed bed or in a fluidized bed.

30 According to the method selected, recourse may then be had respectively to an apparatus of the type of that shown diagrammatically in FIG. 1, or to an apparatus of the type of that shown diagrammatically in FIG. 2.

In the two cases, the hydrogen and the methane or 35 other hydrocarbon arrive respectively through the pipes 1 and 2 opening into a single pipe 3 which leads the gaseous mixture inside an enclosure 4 which is heated by heating elements 5.

In the case of FIG. 1, the enclosure 4 is arranged horizontally and the product 6 to be treated is stacked in a thin layer in a container 7 inside this enclosure. The treatment gas comes into contact with the surface of the product 6.

In the case of FIG. 2, the enclosure is arranged vertically, the product 6 forming a fluid bed above the grid 8. This device also enables working in a fixed bed, the treatment gas then passing through the layer of product 6.

The apparatus of FIG. 2 enables the treatment of much larger amounts of product 6 in shorter reaction times, 50 whether in a fixed bed or in a fluid bed, since it achieves a better contact between the product 6 and the treatment gas.

To establish ideas, it is indicated that the duration of the step of simultaneous reduction and carburation is 55 (in the case of treatment in a fixed bed by means of the apparatus of FIG. 1) generally of the order of 10 to 20 hours.

The proportions of hydrogen and of hydrocarbon of the atmosphere used during this step are respectively of the order of 99.0 to 90 and of 1 to 10%. In practice, one adheres to approximately theoretical proportions to avoid cracking of the hydrocarbon.

60 It is noted that the carburation of a mixed hydroxide or oxide accompanied by reduction of one of the metallic elements to the metallic state according to the method according to the invention is easier than a carburation of a simple oxide, always better crystallized, hence less reactive. This is particularly established in the case of the carburation of titanium in the presence, for example, of iron, of nickel or of cobalt: the carbide TiC is then

## 3

formed between 800 and 1000° C. whilst it is impossible to obtain in this range of temperature when there is subjected to the action of the hydrogen-methane mixture, the hydroxide  $Ti(OH)_4$  or the oxide  $TiO_2$ .

The dispersions according to the invention, prepared by means of the abovesaid method, can be used for the practicing of conventional technics of powder metallurgy, by subjecting them to sintering either as they are, or after having mixed them with a powder of the second metal if the proportion of carbide must be reduced in the final material.

In order that the invention may be more fully understood, various examples of the method and products according to the invention are described below, purely by way of non-limiting illustration.

## EXAMPLE 1

In order to prepare a dispersion of chromium carbide in iron containing 95% by weight of iron, one commences by preparing the mixed oxalic complex



obtained by syncrystallization of the complex oxalates of each of the two metals.

The product thus obtained is subjected to selective carburation by bringing its temperature to 900° C. at the speed of 250° C./h. in a gaseous current distributed by a mixing metering pump and constituted by hydrogen (21.80 l./h.) and by methane (0.44 l./h.), i.e. containing 2% of methane. After 18 hours of maintenance at 900° C. in the atmosphere considered, it is observed by radiocrystallographic analysis that the product obtained is two-phase and contains also orthorhombic chromium carbide  $Cr_3C_2$  finely dispersed in the  $\alpha$  iron. This product has the form of a fine grey powder.

## EXAMPLE 2

In order to prepare a dispersion of chromium carbide in iron, containing 60% by weight of iron, one starts by preparing the mixed oxalic complex of the desired composition as indicated in Example 1.

The product thus obtained is subjected to carburation at 900° C. under conditions of temperature and gaseous flow given in Example 2. After 16 hours of maintenance at 900° C. in the atmosphere considered, radiocrystallographic analysis reveals the presence of a hexagonal single carbide  $Cr_7Cr_3$  dispersed in the  $\alpha$  iron.

## EXAMPLE 3

In order to prepare a dispersion of titanium carbide in cobalt, containing 70% by weight of cobalt, one starts by preparing a co-precipitate of hydrated oxides, in the following manner: there is added simultaneously, but separately and drop by drop, an aqueous solution of 69.1 g. of cobalt nitrate  $Co(NO_3)_2$ , 6H<sub>2</sub>O and 23.2 g. of titanyl sulfate  $TiOSO_4$ , 4H<sub>2</sub>O and a three times normal solution of soda in about one litre of water stirred vigorously in a Pyrex reactor of two litres capacity. The simultaneous precipitation of the two hydroxides takes place drop by drop; the very fine precipitated obtained is filtered, washed with boiling water until disappearance of sulfate and sodium ions, and dried for 20 hours in the oven at 110° C.

The product thus obtained, finely ground, is subjected to simultaneous reduction and carburation by bringing its temperature to 800° C. at the speed of 250° C./h. in a gaseous current constituted of hydrogen (21.80 l./h.) and of methane (1.15 l./h.), i.e. containing 5% of methane. After 16 hours of maintenance in the atmosphere considered, radiocrystallographic analysis confirms the obtaining of a fine dispersion of titanium carbide  $TiC$  in cubic  $\beta$  cobalt. The titanium carbide thus obtained at 800° C. is fine grained, as shown by the wide diffraction lines.

## 4

## EXAMPLE 4

In order to prepare a dispersion of titanium carbide in nickel, containing 90% by weight of nickel, one starts by preparing the co-precipitate of the two hydrated oxides according to the method of operation described in Example 3, by using a saline solution of nickel nitrate and titanyl sulfate.

The compound thus obtained is subjected to simultaneous reduction and carburation by bringing its temperature to 880° C. in a gaseous current constituted by hydrogen (21.80 l./h.) and methane (0.56 l./h.) containing 2.5% of methane. After 16 hours of maintenance in the atmosphere concerned, there is obtained a fine dispersion of the carbide  $TiC$  in metallic nickel.

## EXAMPLE 5

In order to prepare a dispersion of vanadium carbide in cobalt, containing 80% by weight of cobalt, one starts by preparing the co-precipitate of the two hydrated oxides according to the method of operation described in Example 3, by making a precipitation from a saline solution of cobalt nitrate and vanadyl sulfate with a solution of commercial ammonia three times diluted. The precipitation having taken place, it is brought to boiling to restore it to pH 7 and to destroy the vanadate which could have formed.

The compound thus obtained is subjected to simultaneous reduction and carburation by bringing its temperature to 800° C. in a gaseous current of hydrogen (21.80 l./h.) and of methane (1.15 l./h.), i.e. containing 5% of methane. After 14 hours of maintenance at 800° C. in the atmosphere considered, there is obtained a fine dispersion of vanadium carbide  $VC$  in cubic  $\beta$  cobalt.

## EXAMPLE 6

In order to prepare a dispersion of vanadium carbide in iron, containing 80% by weight of iron, one starts by preparing the co-precipitate of the two hydrated oxides according to the operational method described in Example 3, by precipitating from a saline solution of ferric nitrate and vanadyl sulfate with a commercial solution of ammonia diluted three times.

The compound thus obtained is subjected to a simultaneous reduction and carburation by bringing its temperature to 920° C. in a gaseous current of hydrogen (21.80 l./h.) and methane (0.44 l./h.), i.e. containing 2% of methane.

After 20 hours of maintenance at 920° C., radiocrystallographic analysis shows the presence of very little  $\alpha$  iron, of cementite  $Fe_3C$  and of cubic vanadium carbide  $VC$ . Baking of the preceding product under hydrogen (15 l./h. approximately) enables the cementite to be destroyed and there is obtained after 14 hours of baking at 920° C.  $\alpha$  iron, very little  $Fe_3C$  and the carbide  $VC$  finely dispersed. A further baking for 13 h. at 920° C. under hydrogen then leads to the desired product, a dispersion of vanadium carbide in the  $\alpha$  iron.

## EXAMPLE 7

In order to prepare a dispersion of niobium carbide in iron, containing 70% by weight of iron, one starts by preparing an intimate mixture obtained by co-evaporation of the complex oxalates  $(NH_4)_3[Fe(C_2O_4)_3]$  and  $(NH_4)_3[NbO(C_2O_4)_3]$ .

The mixture thus obtained is subjected to a simultaneous reduction and carburation by bringing its temperature to 900° C. in a gaseous current of hydrogen (21.80 l./h.) and of methane (0.44 l./h.), i.e. containing 2% of methane. After 15 hours of maintenance at 900° C., there is obtained a dispersion of  $NbC$  carbide in  $\alpha$  iron.

## EXAMPLE 8

In order to prepare a dispersion of a solid solution of 75 titanium carbides and of tantalum in cobalt, containing

90% by weight of cobalt, one starts by preparing an intimate mixture obtained by co-evaporation of the oxalates  $\text{CoC}_2\text{O}_4$ ,  $(\text{NH}_4)_2[\text{TiO}(\text{C}_2\text{O}_4)_2]$  and



in suitable proportions, and corresponding to the atomic ratio  $\text{Ti}/\text{Ta}=1$ .

The compound thus obtained is subjected to simultaneous reduction and carburation by bringing its temperature to  $950^\circ \text{C}$ . in a gaseous current of hydrogen (21.50 l./h.) and of methane (0.44 l./h.), i.e. containing 2% of methane. After 15 hours of maintenance at  $950^\circ \text{C}$ . in the atmosphere considered, radiocrystallographic analysis indicates the presence of the solid solution of the carbides  $\text{TiC}$  and  $\text{TaC}$  dispersed in a mixture of hexagonal  $\alpha$  cobalt and of cubic  $\beta$  cobalt.

#### EXAMPLE 9

In order to prepare a dispersion of a solid solution of carbides of titanium and of niobium in iron, containing 80% by weight of iron, one starts by preparing an intimate mixture obtained by co-evaporation of the oxalates  $(\text{NH}_4)_3[\text{Fe}(\text{C}_2\text{O}_4)_3]$ ,  $(\text{NH}_4)_3[\text{TiO}(\text{C}_2\text{O}_4)_2]$  and  $(\text{NH}_4)_3[\text{NbO}(\text{C}_2\text{O}_4)_3]$  in suitable proportions and corresponding to the atomic ratio  $\text{Ti}/\text{Nb}=1$ .

The compound thus obtained is subjected to simultaneous reduction and carburation by bringing its temperature to  $1050^\circ \text{C}$ . in a gaseous current of hydrogen (21.80 l./h.) and of methane (0.22 l./h.), i.e. containing 1% of methane. After 15 hours of maintenance at  $1050^\circ \text{C}$ . in the atmosphere considered, radiocrystallographic analysis indicates the presence of the solid solution of  $\text{TiC}$  and  $\text{NbC}$  carbides, dispersed in  $\alpha$  iron

#### EXAMPLE 10

In order to prepare a dispersion of chromium carbide  $\text{Cr}_3\text{C}_2$  in copper, containing 60% by weight of copper, one starts by preparing the starting compound i.e. an intimate mixture obtained by co-evaporation of a solution of the citrates of copper and of chromium. This solution is obtained by heating under reflux, for two hours, an aqueous solution of diammonium citrate in excess to which there is added copper powder, chromic anhydride  $\text{CrO}_3$ , and a little oxygenated water. It is filtered to eliminate the last traces of copper not attacked, and the filtrate is evaporated on a sand bath.

The compound thus obtained, finely ground, is first subjected to oxidation in air, for 12 hours at  $660^\circ \text{C}$ ., which leads to an intimate mixture of cupric oxide  $\text{CuO}$  and of cupric chromite  $\text{CuCr}_2\text{O}_4$ . This mixture, finely ground, is then subjected to simultaneous reduction and carburation, by bringing its temperature to  $1000^\circ \text{C}$ . in a gaseous current of hydrogen (21.50 l./h.) and of methane (0.22 l./h.) i.e. containing 1% of methane. After 15 hours of maintenance at  $1000^\circ \text{C}$ . in the atmosphere considered, radiocrystallographic analysis confirms the obtaining of a dispersion of chromium carbide  $\text{Cr}_3\text{C}_2$  in copper.

#### EXAMPLE 11

In order to prepare a ferronickel alloy with 48% by weight of iron and 52% of nickel, containing 3% by weight of vanadium carbide finely dispersed, one commences by preparing the starting product, i.e. a co-precipitate of the three hydrated oxides according to the method of operation described in the Example 3, by making a starting precipitation from a saline solution of ferric nitrate, of nickel chloride and of vanadyl sulfate with 25% ammonia, operating at pH 7.5.

The compound thus obtained is subjected to simultaneous reduction and carburation by bringing its temperature to  $950^\circ \text{C}$ . in a gaseous current of hydrogen (21.80 l./h.) and of methane (0.44 l./h.) i.e. containing 2% of methane. After 15 hours of maintenance at this temperature in the atmosphere considered, radiocrystallographic analysis shows that there has been obtained a

dispersion of vanadium carbide  $\text{VC}$  in the ferronickel of cubic structure with centered faces, approximating to  $\gamma$  iron, of parameter  $a=3.585 \text{ \AA}$ .

#### EXAMPLE 12

5 In order to prepare a dispersion of 3% by weight of titanium carbide in a nickel-cobalt alloy of composition by weight 90% Ni-10% Co, one starts by preparing the co-precipitate of the three hydrated oxides according to the method of operating described in Example 3, by effecting a precipitation from a saline solution of the chlorides of nickel and cobalt and of titanyl sulfate in suitable proportions, with three times normal soda.

10 The compound thus obtained is subjected to simultaneous reduction and carburation by bringing its temperature to  $1020^\circ \text{C}$ . in a gaseous current of hydrogen (21.80 l./h.) and of methane (0.22 l./h.) i.e. containing 1% of methane. After 16 hours of maintenance at  $1020^\circ \text{C}$ . in the atmosphere considered, radiocrystallographic 15 analysis confirms the obtaining of a nickel- $\beta$  cobalt alloy of center faced cubic structure, very close to that of nickel, containing a dispersion of titanium carbide  $\text{TiC}$ .

#### EXAMPLE 13

20 25 In order to prepare a refractory composition based on titanium carbide, containing 6% by weight of cobalt usable as binder phase in sintering, one starts by preparing a co-precipitate of the two hydrated oxides according to the operational method described in Example 3, 30 by effecting a precipitation from an aqueous solution of titanyl sulfate and of cobalt chloride in suitable proportions, with 25% ammonia. During the whole of the operation the pH must not exceed 8.

35 The compound thus obtained is subjected to simultaneous reduction and carburation by bringing its temperature to  $1030^\circ \text{C}$ . in a current of hydrogen (21.80 l./h.) and of methane (0.22 l./h.) i.e. containing 1% of methane. After 20 hours of maintenance at  $1030^\circ \text{C}$ . in the atmosphere considered and cooling, there is obtained 40 a grey-black powder. Radiocrystallographic analysis confirms the presence of titanium carbide  $\text{TiC}$  and of a binding phase of center faced cubic  $\beta$ -cobalt.

45 As is self-evident, the invention is in no way limited to those of its methods of application, nor to those of its methods of production of its various parts, which have been more particularly indicated; it embraces, on the contrary, all variations.

We claim:

1. Process of preparing a dispersion of at least one 50 carbide in a metallic base, said carbide being in the form of particles distributed uniformly in the midst of elementary grains of said base comprising subjecting at least one first metal from which the carbide is to be formed selected from the group consisting of Ti, V, Nb, Ta and Cr, and at least one second metal selected from the group consisting of Fe, Co, Ni, Cu, Zn, Cd, Ag, Sn, Pb, Bi, Ge and Tl, said metals being in the form of a coprecipitate of hydroxides or a mixed complex thereof in an atmosphere of hydrogen and hydrocarbon to a temperature 55 sufficient to permit simultaneous reduction and carbidization of said coprecipitate or mixed complex and less than  $1100^\circ \text{C}$ ., for a time sufficient to achieve the reduction of all the oxides and the carbidization of said first metal.

2. Method according to claim 1, wherein said metal 60 of the dispersion is an alloy.

3. Method according to claim 1, wherein said hydrocarbon is methane.

4. Method according to claim 1, wherein the heating is effected at a speed of the order of 100 to  $400^\circ \text{C}/\text{hour}$ .

70 5. Method according to claim 1, wherein that the step of simultaneous reduction and carburation is effected in a fixed bed.

6. Method according to claim 1, wherein the step of simultaneous reduction and carburation is effected in a fluidized bed.

7. Method according to claim 5, wherein the duration of the step of simultaneous reduction and carburation is of the order of 10 to 20 hours.

8. Method according to claim 1, wherein the proportions of hydrogen and of hydrocarbon of the atmosphere used during the step of simultaneous reduction and carburation are respectively of the order of 99 to 90 and 1 to 10%.

9. Method according to claim 1, wherein the carbide of the second metal is stable under the conditions of simultaneous carburation and reduction, and said step is followed by a supplementary treatment of reduction in

pure hydrogen at the same temperature for a time sufficient to completely reduce the carbide of said second metal.

**References Cited**

**UNITED STATES PATENTS**

|           |         |                   |       |           |
|-----------|---------|-------------------|-------|-----------|
| 3,013,875 | 12/1961 | Triffleman        | ----- | 75-0.5 AC |
| 3,377,141 | 4/1968  | Hardy et al.      | ----- | 75-0.5 BC |
| 3,399,051 | 8/1968  | Hardy et al.      | ----- | 75-0.5 A  |
| 3,337,327 | 8/1967  | Jordan et al.     | ----- | 75-0.5 AA |
| 3,024,110 | 3/1962  | Funkhouser et al. | ----- | 75-206    |

WAYLAND W. STALLARD, Primary Examiner